

# United States Patent

[11] 3,542,114

[72] Inventors Roy E. Ferree;  
Edward P. Vincent, Valencia, Pennsylvania  
[21] Appl. No. 719,218  
[22] Filed April 5, 1968  
Continuation-in-part of Ser. No. 627,283,  
March 31, 1967, abandoned.  
[45] Patented Nov. 24, 1970  
[73] Assignee Eastern Splash Mats, Incorporated  
Valencia, Pennsylvania

|           |         |                 |            |
|-----------|---------|-----------------|------------|
| 2,923,041 | 2/1960  | Ryznar .....    | 164/72     |
| 3,322,518 | 5/1967  | Hammerton ..... | 44/7       |
| 3,376,914 | 4/1968  | Emmott .....    | 164/67X    |
| 1,752,725 | 4/1930  | Braden .....    | 106/38.25  |
| 2,256,832 | 9/1941  | King .....      | 106/38.25X |
| 2,432,702 | 12/1947 | Wallace .....   | 106/38.8   |
| 2,469,908 | 5/1949  | Wallace .....   | 106/38.8   |
| 2,476,933 | 7/1949  | Wallace .....   | 106/38.25  |
| 2,558,402 | 6/1951  | Wallace .....   | 106/38.8   |

## FOREIGN PATENTS

|         |         |                     |        |
|---------|---------|---------------------|--------|
| 524,917 | 12/1953 | Belgium .....       | 164/74 |
| 986,422 | 3/1965  | Great Britain ..... | 164/74 |
| 254,159 | 7/1926  | Great Britain ..... | 164/42 |

## OTHER REFERENCES

"Processing Molding Sand" By Harry W. Dietent, Transactions of The American Foundrymen's Society Vol. 62, (1954), p. 8 relied on.

Primary Examiner—J. Spencer Overholser  
Assistant Examiner—V. Rising  
Attorney—William J. Ruano

[52] U.S. Cl. 164/74,  
106/38.25, 106/38.8, 117/5.1  
[51] Int. Cl. B22c 3/00,  
B22d 27/00  
[50] Field of Search 164/74, 72,  
73, 67, 42US, 121; 106/38.25, 38.8; 117/5.1

[56] References Cited

### UNITED STATES PATENTS

|           |         |                    |         |
|-----------|---------|--------------------|---------|
| 1,751,038 | 3/1930  | Hoy .....          | 164/67  |
| 1,849,767 | 3/1932  | Michel .....       | 164/42  |
| 1,868,453 | 7/1932  | Wood .....         | 164/42  |
| 1,868,454 | 7/1932  | Wood .....         | 164/42  |
| 1,868,455 | 7/1932  | Wood .....         | 164/42  |
| 1,868,456 | 7/1932  | Wood .....         | 164/42  |
| 1,868,457 | 7/1932  | Wood .....         | 164/42  |
| 2,236,119 | 3/1941  | Craig et al. ..... | 164/42  |
| 2,245,651 | 6/1941  | Craig et al. ..... | 164/72X |
| 2,430,655 | 11/1947 | Wallace .....      | 164/74  |

**ABSTRACT:** This invention relates to a method of purifying, reducing surface imperfections and of lubricating the outer surface of an ingot to facilitate removal from the mold, comprising reacting naphthalene in powder or liquid form by pouring molten metal thereon in an ingot mold or pouring the naphthalene during teeming thereby creating an inert and dense cloud of carbonaceous smoke that will rise in the mold and prevent oxidation and that will coat the inner surface of the mold and outer surface the ingot. Various organic and inorganic compounds are mixed in specified proportions with the naphthalene.



**METHOD FOR PURIFYING AND IMPROVING THE SURFACE QUALITY OF AN INGOT**

This invention relates to a novel method of purifying, reducing surface imperfections and lubricating an ingot as molten metal is poured into the mold. This invention is a continuation-in-part of my U.S. Pat. application Ser. No. 627,283, filed March 31, 1967, now abandoned.

An outstanding disadvantage of presently used methods of casting ingots is that imperfections are formed on the outer surface thereof, many of which are caused by abrasion or friction resulting from removal of the ingot from the mold and from scabs and splashes reduced or eliminated by this invention.

Another disadvantage is that oxidation of molten steel takes place during the teeming of this metal since the surrounding atmosphere contains oxygen.

An object of the present invention is to overcome the above-named disadvantages of present methods and to provide a novel method for greatly reducing surface imperfections of the ingot and at the same time facilitating removal of the ingot by lubricating the inner surface of the mold and outer surface of the ingot as the result of the teeming process.

A more specific object of the invention is to pour molten metal, such as molten steel, into an ingot mold which contains naphthalene mixed with organic or inorganic compounds on the bottom, or on its inner surfaces, or to pour the naphthalene mixture during teeming so as to facilitate removal and greatly enhance the quality of the outer surface of the ingot by creating an inert atmosphere that eliminates oxidation of the molten steel.

The term "naphthalene" as used in my disclosure is the material "naphthalene" described at page 445 of the 4th Ed. of HACKH'S CHEMICAL DICTIONARY, copyright 1969 by McGraw-Hill, Inc.,.

Other objects and advantages of the invention will become more apparent from a study of the following description.

A mold coating, embodying the present invention, may be manufactured by employing at least 70 percent naphthalene and the remainder of other organic or inorganic materials which serve as binders, as stabilizers, as coloring agents, or as release agents, parting media and deoxidizers. A suitable range of naphthalene per ingot ton of the ingot cast is from about 1/16 pound to about 5 pounds. This naphthalene could be used either as a dry powder or as a liquid which is then allowed to solidify into a solid mass.

We have conducted successful tests involving the addition, in amounts of 1 to 30 percent by weight to the naphthalene of each of the following organic compounds: graphite; Gilsonite; petroleum coke; powdered coke; coke breeze; coal; pitch (in many forms); tar (in many forms); and sizing of particles is not critical.

We have also conducted other successful tests in which the following inorganic compounds were added to naphthalene:

lime- 1 to 15 percent; silicia- 1 to 7½ percent; clay- 1 to 10 percent; iron oxide- 1 to 15 percent and a binder, namely, sodium silicate ½ to 4½ percent.

Tests indicate inorganic additions must be in a finely divided form, such as silica flower, 200 mesh by down. The largest particle size experimented with so far has been 100 mesh and down. It appears that coarser sizes will give less satisfactory results.

The naphthalene powder or liquid mixture so formulated is introduced into the ingot mold just prior to pouring. It may be deposited on the bottom or floor of the mold or on the entire inner surface. When this material is contacted by the molten steel it begins to generate and pour forth a dense cloud of carbonaceous smoke that rises in the mold on top of the molten steel. This reaction imparts, simultaneously, a coating on the outer surface of the ingot and on the inner surface of the ingot mold, at the same time, provides an inert atmosphere that prevents oxidation of the molten steel during the teeming process, therefore greatly enhances the purity or quality of the finished steel ingot. The net result is also a substantial reduction in surface imperfections of the ingot due to the inability of the splash or scab to cling to the mold wall, as well as lubrication of the outer surface of the ingot and inner surface of the mold which will facilitate removal of the solidify ingot from the mold and further reduce imperfections otherwise formed on the surface of the ingot as a consequence of abrasion or friction. Thus the surface quality and the quality of the interior of the ingot are greatly enhanced and, as a consequence, all losses in the further processing or finishing of the steel are reduced.

Although naphthalene has been given as an example of a material that will generate a carbonaceous cloud of smoke as the result of the teeming process when used alone or mixed with organic or inorganic materials, other derivatives of naphthalene or other equivalent materials will be readily suggested to those skilled in the art as the result of the present description, but which materials are considered within the spirit and scope of the present invention.

While I have described several embodiments of my invention, it will be understood that these are by way of illustration only, and that various changes and modifications may be made within the contemplation of my invention and within the scope of the following claims.

We claim:

1. The method of purifying, reducing surface imperfections and lubricating an ingot comprising: introducing into an ingot mold just prior to pouring a composition consisting essentially of at least 70 percent naphthalene mixed with 1 to 30 percent, by weight, of Gilsonite and teeming molten metal into said mold and into contact with said composition and thereby causing said composition to react so as to form a dense, continuous, carbonaceous cloud which coats the outer surface of the ingot and inner surface of the mold.